

## UNITED STATES PATENT OFFICE.

ALBERT A. SOMERVILLE, OF FLUSHING, NEW YORK, ASSIGNOR OF TWO-THIRDS TO  
R. T. VANDERBILT COMPANY, INCORPORATED, OF NEW YORK, N. Y., A CORPOR-  
ATION OF NEW YORK.

## OIL COMPOSITION FOR SATURATING CABLE WRAPPINGS.

No Drawing.

Application filed January 8, 1926. Serial No. 80,065.

This invention relates to an improved oil or grease composition for use in saturating the paper or other materials used as a wrapper for electrical cables.

In the manufacture of cables for use as conductors of electrical current, the wrapping of paper or other material is saturated with a suitable oil composition, such as petroleum or grease of suitable consistency by passing the wrapped cable through a hot saturating or impregnating bath of the oil composition. The oil or grease is, in general, such as is not fluid below 30° C. and has a viscosity of not less than 100 seconds at 100° C. as measured by the Saybolt viscosimeter. In the manufacture of continuous lengths of cable, the impregnating bath is maintained at high temperature for long periods of time. The result, however, is that the saturating bath rapidly deteriorates in its insulating properties, and, at more or less frequent intervals of time, it is necessary to remove the bath and replace it with a fresh bath of suitable insulating properties. Moreover, after the impregnating bath is used, and after the wrapped and saturated cable is enclosed in the usual lead casing, the saturating composition undergoes further deterioration under the influence of electrical stress and of the elevated temperatures to which it may be subjected in use.

The present invention provides an improved saturating or impregnating composition which can be used for greatly prolonged periods of time, as compared with the ordinary saturating or impregnating composition, and which is stabilized so that it will resist deterioration, both during the saturating or impregnating operation, and during the subsequent use of the finished cable as an electrical conductor.

According to the present invention, the petroleum or grease composition, which is to be used for saturating the wrappings of cables, has compounded therewith a small amount of a nitrogenous stabilizing agent which will retard or prevent deterioration, both during the saturating treatment and during the subsequent use of the cable as an electrical conductor. When the cable wrapping is saturated with such a stabilized composition, the resulting cable may be considered as a substantially permanent con-

struction with a minimum liability of deterioration of the saturating or impregnating oil composition with which the wrapping is saturated.

The stabilizing materials which are added, in small amounts, to the oil composition used for saturating the wrappings of cables, may be of a somewhat varied character. Of particular advantage are compounds within the group of organic amines, or imines, and particularly condensation products of aldehydes with ammonia or with amines. In general, the compound so added should be non-volatile at the temperature at which the saturating composition is used, and it should also be stable in the sense that it is not decomposed into volatile or objectionable compounds at such temperature of use. The material added should also be soluble in the oil or grease composition to such an extent that it will form a homogeneous admixture therewith. An oil of the general class of petroleum oils and containing a stabilizer comprising specifically the condensation product of an aldehyde and a nitrogenous base is claimed in my copending application Serial No. 103,374, filed Apr. 20th, 1926.

The stabilizing ingredients or ingredient may be added directly to the oil, if readily soluble therein, or the dissolving of the stabilizing material may be promoted by heating, or the material may be first dissolved in a solvent such as benzol, and the benzol solution then added to the oil, with subsequent heating of the composition to drive off the benzol.

The amount of the stabilizing material which is necessary to add is small. In general, a few per cent at most will suffice, and as little as a fraction of a per cent may be sufficient.

The invention will be further illustrated by the following specific examples, but it is intended and will be understood that the invention is illustrated thereby but is not limited thereto.

A mineral oil composition, such as is commonly used for impregnating the paper wrapping of cables, has added thereto a small amount, e. g. 0.5% to 1% of a condensation product of acetaldehyde with anilin, the admixture being promoted by dis-

solving the condensation product in benzol and then intimately admixing the benzol solution with the saturating bath. When the resulting composition is used for saturating the paper wrapping of cables, by passing the cable through the hot saturating bath, the bath will retain high insulating properties for long periods of time. In fact, the bath may increase in its electrical resistivity from that of the original oil being in this respect radically different from the ordinary saturating bath which rapidly deteriorates in its electrical resistivity. Not only is it possible to use the saturating bath for greatly prolonged periods of time, but the resulting cables which have the wrappings saturated with the improved stabilized composition, will likewise resist deterioration in use, thus being a more valuable and improved form of cable construction.

The mineral oil composition used for impregnating cable wrappings may have rosin oil or pine oil added thereto, to impart somewhat different characteristics to it, such as a change in viscosity and flow point. When such oils are added, the nitrogenous stabilizing ingredient or ingredients may be added to a mineral oil or with a pine oil or rosin oil.

Instead of using a condensation product of acetaldehyde and anilin, the condensation product of aldol and alphanaphthylamine can be similarly used.

While I do not wish to limit myself by any theoretical explanations of the action of the stabilizers used in the present invention, yet I believe their actions to be due to prevention of oxidation at the elevated temperatures to which the oils are subjected in use. Although the stabilizing ingredients are used only in very small amounts, not usually exceeding about 2%, and in some cases being only a fraction of a percent, nevertheless they appear to impart remarkable stability to the oil compositions from the standpoint of preventing the usual rapid deterioration of such oil compositions at elevated temperatures.

Instead of using the particular stabilizing materials above mentioned, other nitrogenous stabilizing materials can be used. Among these may be mentioned other members of the group of organic amines and imines, such as homologues of anilin, benzidin and its homologues, paraphenylenediamine, and other aromatic diamines, alpha or beta naphthylamine, etc. Among the condensation products of aldehydes and ammonia or amines may be mentioned, in addition to those above given, other condensa-

tion products of aldehydes, such as formaldehyde, acetaldehyde, benzaldehyde, furfuraldehyde, etc., with ammonia or with amines such as anilin and its homologues, alpha or beta naphthylamine, etc. Examples of such condensation products are the condensation product of aldol with alpha naphthylamine, the condensation product of acetaldehyde with anilin (both the acid and the neutral condensate), the condensation product of formaldehyde with anilin, the condensation product of acetaldehyde with ortho or para toluidine, etc., the condensation product of furfuraldehyde with ammonia or with aniline or orthotoluidine, etc.

It will thus be seen that the present invention is of more or less general application to petroleum oil compositions of the kind used for saturating cable wrappers, imparting to these oils improved stabilized properties such that they resist the usual deterioration and can be used for long periods of time without losing their valuable electrical insulating properties. It will also be seen that, in the case of the cables which have their wrappings saturated with the new composition, the resulting cables are themselves of an improved character, because of the stabilized nature of the saturating composition with which the cable wrappings are saturated.

I claim:—

1. An improved composition for saturating cable wrappings, comprising petrolatum and a small amount of a nitrogenous stabilizing material which retards loss of electrical resistivity of the saturating material at an elevated temperature during the saturating of the cable wrappings, and subsequently in the use of the cables as electrical conductors.

2. An improved composition for saturating cable wrappings, consisting of a petroleum oil of suitable consistency and a small amount of an inert nitrogenous stabilizing material substantially free from acid radicals which retards loss of electrical resistivity of the saturating material at an elevated temperature during the saturating of the cable wrappings, and subsequently in the use of the cables as electrical conductors.

3. In a process for treating cable wrappings, the step of impregnating the cable wrapping with a composition comprising a petroleum oil of suitable consistency and a condensation product of a nitrogenous base and a carbonyl compound.

In testimony whereof I affix my signature.

ALBERT A. SOMERVILLE.